

1  
2,737,463

## METHOD OF COPPERIZING ALUMINUM AND ALUMINUM ALLOYS

Ledra M. Lawton and Stuart T. Ross, Lockport, N. Y., assignors to General Motors Corporation, Detroit, Mich., a corporation of Delaware

No Drawing. Application April 19, 1952,  
Serial No. 283,246

10

10 Claims. (Cl. 117—130)

This invention has to do with the application of metal coatings to metal surfaces and is more particularly concerned with the application of a coating of copper to the surface of aluminum and aluminum alloys.

The usual methods for applying copper to aluminum and its alloys have not been entirely satisfactory. For example, the usual methods of electroplating are not satisfactory for coating aluminum with copper and satisfactory electroplated coatings can be produced only by means of special and rather expensive methods. It also has been proposed heretofore to coat aluminum with copper by contacting the aluminum surface with fused cuprous chloride. However, this method has not proven entirely satisfactory in practice. It has also been desired to produce aluminum having clean coatings of copper thereon, such that the coated metals can be soldered more readily by ordinary methods than can aluminum surfaces.

One object of the present invention is to produce a novel and highly satisfactory method for coating aluminum and its alloys with copper.

Another object is to treat aluminum and aluminum alloy surfaces so that they can be more readily soldered to other metals or may be more readily electroplated with other metals.

Other objects and advantages of the present invention will be more apparent from the following description of specific embodiments of procedure in accordance with the invention.

In accordance with the present invention the surface of an article or base member of aluminum or an aluminum alloy composed preponderantly of aluminum may be coated with an adherent, substantially impervious clean copper coating by a process which includes first coating the article with a slurry consisting of cuprous chloride suspended in rosin which has been plasticized with a terphenyl type compound. The terphenyl type compound and rosin function to keep the cuprous chloride in suspension. After the article has been coated with the slurry as just described, it is treated to remove excess plasticizer to form a dry coating. After this is accomplished the aluminum article with the dry coating is heated to an elevated temperature for a short period of time sufficient to cause the copper to be deposited on the aluminum surface in an adherent form.

In accordance with a preferred embodiment of the invention the slurry consists of two parts by weight of finely divided cuprous chloride and one part by weight of a paste consisting of finely powdered rosin intimately mixed with a terphenyl type compound which may be illustrated by the following formula,  $C_6H_5-C_6H_4-C_6H_5$ . Any one or more of the isomers of terphenyl, singly or in mixtures, may be used. Specific examples are 1,3-diphenyl benzene and 1,4-diphenyl benzene. The preferred composition of the paste consists of 15 parts by weight of finely pulverized rosin and 85 parts by weight of terphenyl as a plasticizer for the rosin. The rosin may be melted and the terphenyl added. The aluminum or aluminum alloy article to be coated with copper has

5 applied to the surface thereof at approximately room temperature (about 70° F.), a coating of the slurry prepared as just described. The coating then is dried as by means of heating to vaporize and drive off excess plasticizer. About 30 to 60 seconds at a temperature of approximately 300° to 350° F. has proven satisfactory in most instances. The article with the dried coating then is heated to a temperature of 750° F. in an oxidizing atmosphere at atmospheric pressure for a short time thereby producing an adherent coating of copper on the article. A time of about 30 seconds or less is all that is necessary. After the copper coating is formed on the aluminum or aluminum alloy article the excess cuprous chloride and rosin and plasticizer, if any, is washed off the copper-coated article. An aqueous solution of potassium chloride or ammonium hydroxide has been found particularly suitable for use in the washing operation.

10 While the foregoing is a specific example of a presently preferred mode of procedure in accordance with the invention, considerable variation in the conditions may be employed with success. For example, the slurry of cuprous chloride and paste consisting of rosin and terphenyl type compound may vary from about five parts by weight of cuprous chloride and one part by weight of the paste of rosin and terphenyl to one part by weight of cuprous chloride and one part by weight of the paste. Also, temperatures higher and lower than approximately room temperature may be employed in the first step of coating the aluminum or aluminum alloy with the slurry consisting of cuprous chloride, pulverized rosin and the plasticizer. Temperatures above 90° F. cause or tend to cause breaking of the suspension. Temperatures as low as 60° F. or even somewhat lower than this may be employed under certain conditions. The temperature employed in the drying step is for the purpose of driving off the excess plasticizer and may be varied as desired with this purpose in mind. The temperature of heating in forming the copper coating may also vary considerably from 750° F. For example, temperatures up to as high as 850° F. may be employed as well as lower temperatures such as 650° F. or even as low as 600° F. under some conditions. Where the higher temperatures are employed it is unnecessary to use as long a time for the heating as where lower temperatures are used. For example, as low as 10 seconds may be used at a temperature of about 800° F. For temperatures as low as 600 or 650° F. it is preferred to employ longer times for the heating step.

15 While very satisfactory results have been obtained by carrying out the heating step in an oxidizing atmosphere it is also contemplated that the heat treatment may be carried out in neutral or reducing atmospheres.

20 In addition to simply forming a coating of copper on aluminum the heat treatment at elevated temperature conditions also causes some diffusion of the copper into the aluminum so that the treated article consists of aluminum or an aluminum alloy having a diffused zone of copper-aluminum alloy and this is covered with a coating of copper and in case the article has been produced in an oxidizing atmosphere a thin outer layer of an oxide of copper.

25 After the excess cuprous chloride and rosin (and plasticizer if any) has been removed as by washing, the aluminum having the copper coating thereon may be soldered to other similarly coated articles or to other metals. Also the copper coated article may be readily electroplated or coated with another metal if desired.

30 Various changes and modifications of the specific embodiments of our invention described herein may be made by those skilled in the art without departing from the spirit and principles of the invention.

We claim:

1. A method of applying a copper coating to a base metal having a surface composed at least preponderantly of aluminum comprising coating said base with a slurry of cuprous chloride suspended in rosin plasticized with a terphenyl type compound, thereafter heating said base and slurry thereon for a time and at a temperature sufficient to volatize excess plasticizer and thereby dry the slurry on said base and then heating the base and dried coating at a higher temperature than the drying temperature and for a time sufficient to form a copper coating on said base.

2. A method of applying a copper coating to a metal base composed at least preponderantly of aluminum comprising coating said base with a slurry of cuprous chloride suspended in rosin plasticized with a terphenyl type compound, said slurry being at a temperature within the approximate range of 60° to 90° F., thereafter heating said base having the coating of the slurry thereon to a temperature and for a time sufficient to drive off excess plasticizer to form a dry coating and thereafter heating the base metal and the dried coating thereon at a temperature within the approximate range of 600° to 850° F. for a time sufficient to form a copper coating on said base.

3. A method of applying a copper coating to a metal base composed at least preponderantly of aluminum comprising coating said base with a slurry of cuprous chloride suspended in rosin plasticized with a terphenyl type compound, said slurry being at a temperature within the approximate range of 60° to 90° F., thereafter heating said base having the coating of the slurry thereon to a temperature of about 300°-350° F. for a time of about 30-60 seconds to form a dry coating and thereafter heating the base metal and the dried coating thereon at a temperature within the approximate range of 600° to 850° F. for a time of about 10 to about 30 seconds.

4. A method of applying a copper coating to a base metal composed at least preponderantly of aluminum comprising coating said base with a slurry of cuprous chloride suspended in rosin plasticized with terphenyl ( $C_6H_5-C_6H_4-C_6H_5$ ), the proportion of cuprous chloride in said slurry ranging from about five parts by weight of cuprous chloride to about one part by weight of the plasticized rosin to one part by weight of cuprous chloride and one part by weight of plasticized rosin, thereafter drying said coating by heating at a temperature on the order of 300° to 350° F. for about 30 to 60 seconds, thereafter heating the base metal and dried coating to a temperature within the approximate range of 600° F. to 850° F. for a period of not over about 30 seconds and thereafter removing any excess cuprous chloride and rosin.

5. A method of applying a copper coating to a base metal composed at least preponderantly of aluminum comprising coating said base with a slurry of cuprous chloride suspended in rosin plasticized with terphenyl ( $C_6H_5-C_6H_4-C_6H_5$ ), the proportion of cuprous chloride in said slurry ranging from about five parts by weight of cuprous chloride to about one part by weight of the plasticized rosin to one part by weight of cuprous chloride and one part by weight of plasticized rosin, said slurry being at a temperature within the approximate range of 60°-90° F., thereafter drying said coating by heating at a temperature on the order of approximately 300° to approximately 350° F. for about 30 to 60 seconds, thereafter heating the base metal and dried coat-

ing to a temperature within the approximate range of 600° F. to 850° F. for a period of about 10 to 30 seconds and thereafter removing excess cuprous chloride and rosin.

5. A method of applying a copper coating to a base metal composed at least preponderantly of aluminum comprising coating said base with a slurry consisting of about two parts by weight of cuprous chloride and one part by weight of a mixture of finely divided rosin and terphenyl ( $C_6H_5-C_6H_4-C_6H_5$ ), said rosin and terphenyl being present in the proportions of about 15 parts by weight of rosin and 85 parts by weight of terphenyl, said slurry being at a temperature within the approximate range of 60-90° F., then heating said base metal to a temperature of approximately 300 to 350° F. for a short period of time sufficient to remove excess terphenyl and form a dry coating on said base, and then heating said base metal with the dried coating thereon to a temperature of approximately 750° F. for a time of approximately 10 to 30 seconds.

7. A method of applying a copper coating to a base metal composed at least preponderantly of aluminum comprising coating said base with a slurry consisting of about two parts by weight of cuprous chloride and one part by weight of a mixture of finely divided rosin and terphenyl ( $C_6H_5-C_6H_4-C_6H_5$ ), said rosin and terphenyl being present in the proportions of about 15 parts by weight of rosin and 85 parts by weight of terphenyl type compound, said slurry being at approximately room temperature, then heating said base metal to a temperature of approximately 300 to 350° F. for about 30 to 60 seconds to remove excess terphenyl and form a dry coating on said base and then heating said base metal with the dried coating thereon to a temperature of approximately 750° F. in an oxidizing atmosphere at atmospheric pressure for a time of approximately 10 to 30 seconds.

8. A method of applying a copper coating to a base metal composed at least preponderantly of aluminum comprising coating said base with a slurry consisting of two parts by weight of finely divided cuprous chloride and one part by weight of a paste consisting of about 85 parts terphenyl ( $C_6H_5-C_6H_4-C_6H_5$ ) and 15 parts by weight of rosin, said slurry being applied to the aluminum at a temperature of about 70° F., thereafter heating the coating for about 30 seconds to a temperature of about 350° F. to remove excess terphenyl and form a dry coating on said base and thereafter heating the base metal with the dried coating thereon in an oxidizing atmosphere at a temperature of about 750° F. at atmospheric pressure for a time of about 30 seconds.

9. A process as in claim 4 in which any excess cuprous chloride and rosin are removed by washing in an aqueous solution of the class consisting of potassium chloride and ammonium hydroxide.

55 10. A process as in claim 8 in which any excess cuprous chloride and rosin are removed by washing in an aqueous solution of the class consisting of potassium chloride and ammonium hydroxide.

60 References Cited in the file of this patent

UNITED STATES PATENTS

|           |                 |               |
|-----------|-----------------|---------------|
| 675,584   | Betts           | June 4, 1901  |
| 1,370,967 | Hommel          | Mar. 8, 1921  |
| 2,331,356 | Swenson         | Oct. 12, 1943 |
| 2,462,631 | Gittings et al. | Feb. 22, 1949 |
| 2,551,712 | Soby            | May 8, 1951   |